

## UNITED STATES PATENT OFFICE.

CHARLES F. RUSSI AND CELEDONIO CADENA, OF SAN ANTONIO, TEXAS.

## ARTIFICIAL FUEL.

SPECIFICATION forming part of Letters Patent No. 727,694, dated May 12, 1903.

Application filed September 29, 1902. Serial No. 125,299. (No specimens.)

*To all whom it may concern:*

Be it known that I, CHARLES F. RUSSI and CELEDONIO CADENA, citizens of the United States, residing at San Antonio, in the county 5 of Bexar and State of Texas, have invented a new and useful Artificial Fuel, of which the following is a specification.

This invention relates to artificial fuel.

The object of the invention is entirely to dispense with the employment of coal, coke, or other carbonaceous substances as a gas-producing element and in lieu thereof to combine elements readily obtainable in nearly all localities in the production of a thoroughly efficient, economical, and highly-combustible fuel.

With these and other objects in view, as will appear as the nature of the invention is better understood, the same consists in the 20 artificial fuel and combination of ingredients composing the same, as will be hereinafter fully described and claimed.

In carrying the invention into effect there is taken of the following ingredients, by 25 weight: sawdust, one-half ( $\frac{1}{2}$ ) part; manure, one and one-half ( $1\frac{1}{2}$ ) parts; sand, three-fourths ( $\frac{3}{4}$ ) part; marl, three-fourths ( $\frac{3}{4}$ ) part; clay, one (1) part, and lime-water. The quantity of lime employed is preferably about 30 thirty-five pounds unslaked white lime to one hundred gallons of water. All of the ingredients are thoroughly mixed, the amount of lime-water employed being just sufficient to render the mass plastic, and the compound 35 is then molded into briquets of suitable size and then dried.

The fuel thus produced may be substituted for ordinary soft or bituminous coal for forge-work or in furnaces of all kinds and is also 40 adaptable for use in heating or cooking stoves of the ordinary construction. It is exceedingly inflammable, and the fire may be started with ordinary kindling-wood. Under combustion it is free from all gases, burns freely

and without formation of clinkers, and bulk 45 for bulk will last longer than ordinary soft coal. It also has the additional advantage of being from twenty-five to thirty per cent. cheaper in price than soft coal, and owing to the cheapness of its ingredients and the 50 readiness with which they may be obtained may be manufactured in almost any locality.

While the proportions of ingredients herein stated are found thoroughly efficient in use, it is to be understood that the invention 55 is not to be limited to those given, as they may be varied if found necessary or desirable and still be within the scope of the invention.

Having thus described the invention, what 60 we claim is—

1. An artificial fuel, consisting of sawdust, manure, sand, marl, clay, and lime-water, substantially in the proportions specified.

2. An artificial fuel, consisting of the following ingredients by weight: sawdust, one-half ( $\frac{1}{2}$ ) part; manure, one and one-half ( $1\frac{1}{2}$ ) parts; sand, three-fourths ( $\frac{3}{4}$ ) part; marl, three-fourths ( $\frac{3}{4}$ ) part; clay one (1) part, and lime-water in quantity sufficient to agglomerate the ingredients into a plastic mass.

3. An artificial fuel composed of the following ingredients by weight: sawdust, one-half ( $\frac{1}{2}$ ) part; manure, one and one-half ( $1\frac{1}{2}$ ) parts; sand, three-fourths ( $\frac{3}{4}$ ) part; marl, three-fourths ( $\frac{3}{4}$ ) part; clay one (1) part, and lime-water in the proportion of thirty-five pounds of unslaked white lime to one hundred gallons of water.

In testimony that we claim the foregoing as 80 our own we have hereto affixed our signatures in the presence of two witnesses.

CHARLES F. RUSSI.  
CELEDONIO CADENA.

Witnesses:

CHARLES K. CRAWFORD,  
JOHN WILKENS, Jr.